

R. A. HADFIELD AND A. G. M. JACK,  
CAPPED ARMOR PIERCING PROJECTILE AND CAP THEREFOR,  
APPLICATION FILED APR. 23, 1914. RENEWED MAR. 30, 1917.

1,310,076.

Patented July 15, 1919.  
2 SHEETS—SHEET 1.

Fig 1.



Fig 2



Witnesses:

J. Rose Mellow  
M. L. Breslin

Inventors:

Robert Abbott Hadfield and  
Alexander George MacKenzie Jack  
By Alfred Wilkupson  
Attorney.

R. A. HADFIELD AND A. G. M. JACK,  
CAPPED ARMOR PIERCING PROJECTILE AND CAP THEREFOR,  
APPLICATION FILED APR. 23, 1914, RENEWED MAR. 30, 1917.

1,310,076.

Patented July 15, 1919.  
2 SHEETS—SHEET 2.

Fig. 3.



*Witnesses:*

J. Macmillan  
M. L. Breslin

*Inventors*

Robert Abbott Hadfield <sup>nd</sup>  
Alexander George Mackenzie Jack  
By Alfred Wilkinson  
Attorney

# UNITED STATES PATENT OFFICE.

ROBERT ABBOTT HADFIELD, OF WESTMINSTER, AND ALEXANDER GEORGE MACKENZIE JACK, OF SHEFFIELD, ENGLAND.

## CAPPED ARMOR-PIERCING PROJECTILE AND CAP THEREFOR.

1,310,076.

Specification of Letters Patent. Patented July 15, 1919.

Application filed April 23, 1914, Serial No. 833,873. Renewed March 30, 1917. Serial No. 158,731.

To all whom it may concern:

Be it known that we, Sir ROBERT ABBOTT HADFIELD, knight, F. R. S., and ALEXANDER GEORGE MACKENZIE JACK, subjects of the 5 King of Great Britain and Ireland, residing respectively, at Westminster, England, and Sheffield, in the county of York, England, have invented Improvements in or Relating to Capped Armor-Piercing Projectiles and 10 Caps Therefor, of which the following is a specification.

This invention has for object to provide 15 caps for armor piercing projectiles that will enable projectiles fitted therewith to completely perforate hard faced armor plates in a more reliable and advantageous manner than heretofore usual both when striking normally and obliquely.

For this purpose according to the present 20 invention a cap of the required weight is made of metal or alloy capable of being stiffened or hardened and possessing considerable toughness or strength and subjected to a stiffening treatment such that the 25 metal is caused to gradually increase in stiffness or hardness in a direction from the part thereof directly in front of the point of the projectile to the extreme front end or point of the cap as hereinafter described, the 30 stiffness or hardness at the latter part of the cap approaching in some cases that of the hard face of the armor plate at which a projectile fitted with a cap is to be fired so that upon impact of the capped projectile 35 against the plate the point of the projectile will pass through cap material of gradually increasing stiffness or hardness and will reach and perforate the plate without being suddenly subjected to contact with a surface 40 that is considerably harder than the front end portion of the cap material as has heretofore been usual. As a result, the point of the projectile is supported with a gradually increasing pressure from the moment 45 of impact of the cap against the hard surface of the plate until it enters the plate, the sudden shock which the point of a projectile ordinarily receives when passing through the relatively soft metal of a cap 50 and striking the hard surface of the plate being avoided with advantageous results. A further result of using a cap of the kind referred to is that on impact against a hard faced armor plate, its stiffened or hardened 55 front end point enters or bites into the hard

surface of the armor plate so as to center the capped projectile to some extent and effect an initial perforation, disintegration or fracture of such hard surface so as to relieve the hardened point of the projectile to 60 some extent from this duty and enable it and the remainder of the projectile to finish the work of perforating the plate and remain intact or unbroken or practically unbroken under adverse conditions and also at 65 a lower velocity than would otherwise be possible.

In order to obtain the best results both for normal and inclined fire, not only should the cap be made of metal or alloy capable of 70 being stiffened or hardened and possessing considerable toughness but it should be stiffened in such a manner that it should have a ball hardness at or near the middle or central portion or zone of the axial length 75 of its front end portion of the order of about 350 to 500 on the Brinell ball scale, corresponding to a hardness of about 45 to 60 as determined by the scleroscope, the hardness decreasing from this part rearwardly 80 through what may be called a rearward portion or zone, say to a ball hardness of about 200 to 300, corresponding to say about 30 to 40 as determined by the scleroscope, near to or at a short distance in front of the point 85 of the projectile and increasing from the said part in a forward direction through what may be called a forward portion or zone, say to a ball hardness of from 500 to 600, corresponding to from about 60 to 90 90 by the scleroscope, or even higher, at the extreme front end or point of the cap. Thus it will be understood that the major part of the front end portion of the cap by which is meant that portion that extends 95 beyond a plane that is at right angles to the longitudinal axis of the cap and is at or adjacent to the point of the projectile to which the cap is applied, will be well below a ball hardness of about 600, that is to say a 100 hardness which corresponds to glass scratching hardness, the part having a ball hardness of from 350 up to say 560 being of gradually increasing stiffness while possessing great toughness while if the ball hardness of the 105 extreme front end portion or point of the cap be increased up to 600 or above this portion will be in the condition usually understood and technically known in connection with steel by the term "hardened". In the 110

latter case the front end portion of the cap, as defined will have a stiffened forward portion surmounted by a hardened extreme front end portion or point the extent of 5 which may be varied to suit requirement. If the hardness of the front end portion of the cap from the said central portion or zone increases in a forward direction to the extreme front end or point to a ball hardness 10 terminating substantially below a ball hardness of 600, say to a limit not above 580, that is to say well below glass scratching hardness, then the front end portion of the cap will consist of a metal of gradually increasing 15 hardness varying from a condition of softness and toughness up to a condition of toughness and stiffness but not to a condition corresponding to that understood by the term hardened. In each case however the 20 front end portion of the cap will be of sufficient stiffness and toughness as not to break up so quickly as a cap having a hardened front end portion as heretofore proposed so that it will offer a more effective support to 25 the point of the projectile upon impact against an armor plate or other object, until such point reaches the object, than a cap the front end portion of which is hardened in the ordinary sense of the term.

30 The said cap may advantageously be made of nickel chromium steel containing a substantial amount of carbon, nickel and chromium to enable its front end portion to be stiffened to a suitably high degree and leave 35 the rear end portion relatively soft and tough. For example, good results have been obtained with a cap made of nickel chromium steel of the following approximate composition, namely, carbon .34% (decimal 40 three four per cent.), nickel 3.86% (three decimal eight six per cent.) and chromium 1.78% (one decimal seven eight per cent.). The percentages of carbon, nickel and chromium may however vary from those mentioned 45 by way of example provided sufficient carbon is present to enable the front end of the cap to be stiffened or stiffened and hardened to the required degree. In some cases the carbon may amount to .6 to 50 .7% (decimal six to decimal seven per cent.).

In some cases the cap may be of wrought iron or mild steel having a cemented front end portion.

The front end portion of the cap, which 55 may be of conical or pointed shape, or of rounded or of other desired shape, is stiffened to the required varying degrees by heating it to a suitable temperature and then quenching it in a cooling medium.

60 In the case of a cap made of nickel chromium steel of the above mentioned composition, the front end portion of the cap may be heated say to a temperature of about 850° C., and then dipped to a suitable depth 65 into water or other suitable quenching me-

dium and allowed to remain there until it attains the desired stiffness, such as that hereinbefore mentioned, the stiffness gradually decreasing toward the part thereof that will be adjacent to the point of the 70 projectile with which it is to be used, in such manner that the cap material in the neighborhood of the hard pointed front end portion of the projectile is soft and tough, or comparatively so.

75 For a cap suitable for a four and one eighth inch armor piercing projectile and having an axial thickness through its front end portion of about one inch, good results have been attained by heating the front end 80 portion of the cap to a temperature of about 850° C. and stiffening the same in ordinary cold water to a depth of about half an inch; in the case of a cap having an axial thickness of about one and a half inches by stiffening 85 the front end portion of the cap to a depth of about five eighths of an inch and in the case of a cap having an axial thickness of about five eighths of an inch by stiffening the front end portion of the cap 90 to a depth of about half an inch. By stiffening the cap in this way by dipping, it is found to have several zones of varying degrees of hardness, that is to say a front end zone having a ball hardness of 400 and upward, an adjacent rear zone having a decreasing ball hardness of from 400 to 300, and another and adjacent rear zone having a decreasing ball hardness of from about 300 to about 200 at or near the point of the 100 projectile, the remainder or rear end portion of the cap having a ball hardness of about 200. The axial thicknesses through the front end portion of the caps mentioned above are given as examples only and can 105 be increased or decreased to suit requirement and the caliber of the projectiles with which the caps are to be used but not necessarily in direct proportion to the calibers of the projectile.

110 In the accompanying drawings Figures 1, 2 and 3 are sectional elevations showing capped projectiles embodying the present invention.

Figs. 1 and 2 show projectiles *a* each 115 fitted with a cap *b* of ogival shape with a conical or pointed front end made according to the present invention and having a front end portion the axial thickness of which can be made of different lengths as 120 indicated by the dotted lines *b*<sup>1</sup>, *b*<sup>2</sup> and *b*<sup>3</sup>, the cap in Fig. 1 being shown fitted to a projectile the ogival shaped head portion of which has a radius of curvature approximately equal to two calibers of the projectile while the cap in Fig. 2 is shown fitted to a projectile the head portion of which has a smaller radius of curvature.

125 In a cap constructed and stiffened as described, the amount of material having a 130

ball hardness of 250 and over may constitute the whole or practically the whole portion of the cap in front of the point of the projectile.

- 5 Caps made as hereinbefore described may advantageously be subjected to a preliminary heat treatment before being subjected to the stiffening treatment proper. Thus, the nickel chromium steel cap, in the rough 10 forged shape, may be heated all over to about 800° to 850° C., then quenched all over in oil, water or other suitable medium to a temperature of under 400° C., then reheated to about 740° C. and allowed to cool 15 below 400° C., then reheated to about 600° C. and then finally quenched all over in water. The cap is then machined to the required shape after which its front end portion is heated say to about 850° C. and stiffened in 20 the manner hereinbefore described.

When a cap according to the invention is made of wrought iron or soft steel with a cemented front end portion, the cementation process should be carried out in such a manner 25 as to impregnate the greater part of the front end portion of the cap with a suitable amount of carbon such as indicated in connection with the nickel chromium steel hereinbefore referred to. Such a cap may be 30 stiffened or hardened in the manner hereinbefore described for the caps made of nickel chromium steel.

With the object of increasing the lateral support offered by the cap to the pointed 35 end portion or nose of the projectile at the critical moment, namely when the point or nose reaches the armor plate and this without materially increasing the weight of the cap, the ogival or other shaped forward end 40 portion of the cap may be provided intermediate of its front and rear parts with an external annular circumferential bead or ridge which may be of curved outline in cross section. Fig. 3 is a sectional elevation 45 showing a projectile *a* fitted with an ogival shaped cap *b* provided with a bead or extension at *c* such as referred to.

In modern armor piercing projectiles designed for angle attack the weight of the 50 cap usually forms a considerable proportion of the total weight of the capped projectile—it may be say about 15% thereof—with the result that the striking energy of the projectile itself, available for effecting 55 perforation of an armor plate, after impact and dispersal of the cap, is thereby very considerably less than the total initial striking energy of the combined projectile and cap.

60 One of the objects of the present invention is therefore to provide a capped projectile that can perforate hard faced armor plate without becoming broken up, or broken up to such an extent as to seriously detract 65 from its effective action, either when strik-

ing the plate normally or obliquely under difficult conditions and wherein the weight of the cap relatively to the total weight of the capped projectile shall be smaller than usual so that for any given weight of capped 70 projectile the projectile proper can be made of relatively greater weight and strength and will consequently possess, after impact and dispersion of the cap, greater energy and efficiency than usual, which shall be 75 available for enabling it to better perforate the armor plate and yet remain in an intact or not seriously broken up condition.

To this end an armor piercing projectile is provided with a cap having a stiffened or 80 hardened front end portion and a relatively soft rear portion in contact with the hard front end portion of the projectile as hereinbefore described and made of a weight of the order of from about five to twelve per cent. 85 of the weight of the combined projectile and cap. In the case of an armor piercing projectile of about four and one eighth inches diameter, good results have been obtained with hardened caps such as hereinbefore described having weights varying from as low 90 as twenty-three up to sixty ounces, constituting from about 4.5% to 12% of the weight of the combined projectile and cap.

Where necessary, a hollow point or air 95 deflector of known kind may be applied over the front end portion of the cap so as to give the capped projectile the necessary contour but the use of such a hollow point or air deflector forms no part of the present invention. 100

What we claim is:—

1. An armor piercing projectile fitted with a cap having its front end portion made of gradually increasing stiffness, as 105 distinguished from being hardened, in a forwardly extending direction from the part thereof in front of the point of the projectile.

2. An armor piercing projectile fitted with a cap made of nickel chromium steel and of gradually increasing stiffness, as distinguished from being hardened, in a forwardly extending direction from the part 110 thereof in front of a transverse plane passing through the cap near the point of the projectile as set forth.

3. A cap for armor piercing projectiles having a hardened front portion gradually diminishing in hardness toward the rear, 115 said cap having a hardness of from 350 to 500 ball hardness adjacent the center of the axial length of its front end portion, the hardness increasing therefrom forwardly to a hardness of from 500 to 600, and diminishing from said center rearwardly to a hardness of from about 300 to 200, substantially as described and shown.

4. A cap for an armor piercing projectile made of nickel chromium steel and of gradu- 130

- ally increasing hardness from the rear toward the front end, the steel of said cap being low in carbon, having nickel above about three per cent. and chromium above 5 about one per cent.
5. For an armor piercing projectile, a cap having its front end portion made of gradually increasing stiffness or hardness in a direction from the part thereof that will be in 10 front of and near to the point of the projectile to which it is to be fitted and provided with an external annular circumferential bead or extension, the diameter through said beaded portion being substantially less 15 than the maximum diameter of the cap, substantially as described.
6. An armor piercing projectile fitted with a cap the front end portion of which is made of gradually increasing stiffness in a 20 forward direction, as set forth, and the weight of which cap is of the order of from about four and a half to twelve per cent. of the weight of the combined projectile and cap.
- 25 7. An armor piercing projectile provided with a cap having its front portion gradually increasing in stiffness forward from the part adjacent the point of the projectile, and the extreme front end point or tip very 30 hard, approaching in hardness the hard face of the armor plate.
8. A cap for an armor piercing projectile having a relatively soft rear portion, a front portion gradually increasing in hardness 35 toward the front end, and the extreme point or tip made very hard.
9. An armor piercing projectile provided with a cap having its front end portion of gradually increasing stiffness toward the 40 front, said cap being made of nickel chromium steel or of wrought iron or mild steel, the extreme front point or tip having been hardened by cementation before the remainder of the cap has been stiffened.
- 45 10. A cap for armor piercing projectile, having successive portions or zones of its front end portion, proceeding in a forward direction, of successively increasing degrees of ball hardness increasing from about 200 50 to 300 at the part of the cap adjacent to a transverse plane that would pass through the point of the projectile to which the cap is fitted.
11. A cap for an armor piercing projectile, the front portion of which is of gradually increasing hardness, but having its front end portion stiffened as distinguished from hardened and substantially below a ball hardness of the order of about 600. 55
12. A cap for an armor piercing projectile the portion of which will be forward of the point of the projectile to which the cap is to be fitted is of gradually increasing stiffness in a forward direction, the final degree of stiffness adjacent the front 60 not exceeding that corresponding to a ball hardness of about 560.
13. A cap for an armor piercing projectile having a hardened tip or nose carried by an unhardened but stiffened and toughened 65 front portion.
14. A cap for an armor piercing projectile having its front portion made of gradually increasing stiffness, as distinguished from being hardened, in a forwardly extending 70 direction and having a hardened extreme front tip or nose.
15. A cap for an armor piercing projectile, having a hardened front portion gradually diminishing in hardness toward the 75 rear, said cap having a ball hardness of the order of about 350 adjacent to the center of the axial length of its front end portion, a ball hardness of the order of about 600 or above at the extreme tip and a ball hardness of the order of about 200 to 300 at the 80 rear end of said front portion.
16. A steel cap for armor piercing projectiles containing a substantial amount of carbon, nickel and chromium, to enable its 85 front portion to be stiffened and its rear portion relatively soft.

Signed at Sheffield this 15th day of January, 1914 and at Washington, D. C., U. S. A., this 3rd day of February, 1914.

ROBERT ABBOTT HADFIELD.  
ALEXANDER GEORGE MACKENZIE JACK.

Witnesses to the signature of Sir Robert Abbott Hadfield:

ANSON S. TAYLOR,  
ALFRED WILKINSON.

Witnesses to the signature of Alexander George Mackenzie Jack:

LUTHER J. CARR,  
E. MORTIMER.